

# UNITED STATES PATENT OFFICE.

CHARLES J. REED, OF PHILADELPHIA, PENNSYLVANIA.

## PROCESS OF ELECTROLYTICALLY REMOVING SCALE AND PRODUCING IRON SULFATE.

No. 855,667.

Specification of Letters Patent.

Patented June 4, 1907.

Application filed June 18, 1906. Serial No. 322,270.

*To all whom it may concern:*

Be it known that I, CHARLES J. REED, a citizen of the United States, residing at Philadelphia, in the county of Philadelphia and 5 State of Pennsylvania, have invented certain new and useful Improvements in Processes of Electrolytically Removing Scale and Producing Iron Sulfate, of which the following is a specification.

10 Various electrolytic methods have been proposed for removing the oxid scale from iron sheets, rods and wire. In some of these the iron article is made the anode in an electrolyte of acid or an acid salt. The scale is thus dissolved more rapidly than in the usual 15 pickle bath but the action is apt to be irregular and solution of the iron invariably occurs. Furthermore the gain in time is more than offset by the cost of the electric current. 20 In other proposed methods the iron article is made the cathode in an electrolyte which is neutral, weakly acid or alkaline, for example, a dilute solution of an alkali-metal salt, an acid or an alkali. The removal of scale, 25 however, is slow and irregular, spots of scale being frequently left at various points. Some of the scale is also loosened by the electrolytic hydrogen and drops into the bath. In neutral or alkaline solutions, much of the 30 scale is reduced to metallic iron, producing a rough, irregular surface.

According to the present invention, the iron article is made the cathode in an electrolyte containing sulfuric acid, preferably 35 in strong aqueous solution. The scale is thereby reduced to a lower state of oxidation and electrolytically dissolved with the production of ferrous sulfate. An insoluble anode is employed and sulfur or an oxidizable sulfur compound is supplied to the electrolyte, serving by its oxidation to both de-polarize the anode and replenish the acid in 40 solution.

In the preferred mode of procedure, the 45 electrolyte consists of an aqueous solution of sulfuric acid having a specific gravity of about 1.20, equivalent to an acid content of 27.1 percent. The anode may be of lead and the current density at the cathode from 50 40 to 70 amperes per square foot. The electrolyte is preferably maintained at a temperature of about 60° C. Free sulfur or an oxidizable sulfur-bearing compound, such as a supersulfid of a non-alkali metal, specifically 55 pyrite, marcasite or pyrrhotite, is supplied to or maintained at or near the anode and

the sulfur is oxidized to trioxidat a rate corresponding to the reduction and solution of the scale on the cathode, thus continuously replenishing the electrolyte. A diaphragm cell may be employed, to retain in proximity to the anode any sulfur dioxid resulting from incomplete oxidation of the sulfur whereby it is finally oxidized to trioxid and prevented from interfering with the 65 cathodic reduction. The production of sulfuric acid corresponds to the rate of its consumption by the formation of ferrous sulfate, the electrolyte thus being maintained at the proper concentration. In the case of a diaphragm cell, the concentration of the acid in the catholyte is maintained by diffusion and cataphoresis from the anolyte.

As the amount of iron sulfate in solution approaches saturation, the electrolyte or 70 catholyte is transferred to a shallow pan and allowed to cool. It is preferable to reduce its temperature to about 0° C. by the use of a suitable refrigerant. The iron sulfate crystallizes out and the residual solution is 75 returned to the electrolytic cell, no evaporation or further treatment being required to fit it for continued use as an electrolyte.

The expression "an oxidizable sulfur-bearing material," as used in the claims, is intended to include both free sulfur and sulfur compounds.

I claim:—

1. The process of electrolytically dissolving iron-oxid scale from the surface of metal, 90 which consists in passing an electric current to the metal, as cathode, in an electrolyte containing sulfuric acid and a substance capable of yielding sulfuric acid by oxidation, as set forth.

2. The process of electrolytically dissolving iron-oxid scale from the surface of metal, 100 which consists in passing an electric current to the metal, as cathode, in an electrolyte consisting of a strong aqueous solution of sulfuric acid and containing a substance capable of yielding sulfuric acid by oxidation, as set forth.

3. The process of electrolytically dissolving iron-oxid scale from the surface of metal, 105 which consists in passing to the metal as cathode, in an electrolyte consisting of a heated, strong aqueous solution of sulfuric acid, an electric current of sufficient density to rapidly remove the scale, and maintaining an 110 oxidizable sulfur-bearing material at or in proximity to the anode, as set forth.

4. The process of electrolytically dissolving iron-oxid scale from the surface of metal, which consists in passing to the metal as cathode, in an electrolyte consisting of a heated, strong aqueous solution of sulfuric acid, an electric current of sufficient density to rapidly remove the scale, and maintaining a sulfid of a non-alkali metal at or in proximity to the anode, as set forth.
- 10 5. The process of electrolytically dissolving iron-oxid scale from the surface of metal, which consists in passing to the metal as cathode, in an electrolyte consisting of a heated, strong aqueous solution of sulfuric acid, an electric current of sufficient density to rapidly remove the scale, and maintaining a sulfid of iron at or in proximity to the anode, as set forth.
- 15 6. The process of electrolytically dissolving iron-oxid scale from the surface of metal, which consists in passing an electric current to the metal, as cathode, in an electrolyte containing sulfuric acid and a substance capable of yielding sulfuric acid by oxidation, and recovering the iron sulfate from the resulting solution, as set forth.

7. The process of electrolytically dissolving iron-oxid scale from the surface of metal, which consists in interposing a diaphragm between a catholyte and anolyte containing sulfuric acid, passing an electric current to the metal, as cathode, and supplying an oxidizable sulfur-bearing material to the anolyte, as set forth.

8. The process of electrolytically dissolving iron-oxid scale from the surface of metal, which consists in interposing a diaphragm between a catholyte and anolyte consisting of a heated, strong aqueous solution of sulfuric acid, passing an electric current to the metal, as cathode, supplying an oxidizable sulfur-bearing material to the anolyte, removing and cooling the catholyte, thereby precipitating the ferrous sulfate, and returning the residual solution to the anode compartment, as set forth.

In testimony whereof, I affix my signature in presence of two witnesses.

CHARLES J. REED.

Witnesses:

ROBT. B. FLETCHER,  
M. H. QUINN.